

No. 668,282.

Patented Feb. 19, 1901.

C. G. COLLINS.

## AMALGAMATOR.

(No Model.)



**Witnesses:**

W. Andrew.  
L. M. Matt.

Inventor:  
Caleb G. Collins  
By his Attorney  
George William Smith

# UNITED STATES PATENT OFFICE.

CALEB G. COLLINS, OF WOODMERE, NEW YORK, ASSIGNOR TO CALVIN AMORY STEVENS, OF NEW YORK, N. Y.

## AMALGAMATOR.

SPECIFICATION forming part of Letters Patent No. 668,282, dated February 19, 1901.

Application filed January 4, 1899. Serial No. 701,097. (No model.)

*To all whom it may concern:*

Be it known that I, CALEB G. COLLINS, a citizen of the United States, residing at Woodmere, Queens county, and State of New York, have invented certain new and useful Improvements in Amalgamators, of which the following is a specification sufficient to enable others skilled in the art to which the invention appertains to make and use the same.

10 My invention is designed to effect a more thorough and rapid extraction of metal from the ore or gangue than has heretofore been practicable; and it consists in the special construction and arrangement of parts hereinafter set forth, and particularly pointed out in the claim.

The accompanying drawing represents a vertical section of apparatus designed to give practical effect to my invention.

20 The amalgamating-tank A is preferably, although not necessarily, of cylindrical form, arranged vertically and formed of a metal not affected by mercury.

B is a stand-pipe which extends from near the bottom of the cylinder A to a height sufficient to render gravity available in forcing the ore-pulp introduced through said pipe B into and through the column of mercury in the cylinder A, the level of which mercury is indicated by the line m m. The pipe B is supported so as to be free to rotate upon its longitudinal axes by any suitable mechanical expedient, as by shoulders b b, resting upon the upper ends of the bearings C C. It is provided with a power-pulley W, by which it is rotated, and with a funnel-shaped mouth Q at its upper extremity to facilitate the introduction of the ore or pulp.

25 D represent a series of iron plates or disks secured rigidly to the pipe B and rotating therewith. These plates D are perforated, but the plates are so arranged with relation to each other that the perforations in adjoining plates do not coincide. The series of plates D are designed to be immersed in the mercury. The upper plate D', in addition to being perforated, is provided with a series of iron rods d, extending downward from its under surface to within, say, about 35 an inch of the surface m m of the mercury.

Extending from the side of the cylinder,

near its lower extremity, is a pipe E, projecting upward above the line of mercury in the cylinder A and provided at top with a vessel F for the reception of a solution of sodium salt, such as sodium chlorid. P is a carbon plate situated in said soda-tank F and representing the positive pole or anode of an electrical circuit, of which p is a symbolical representation of the conductor from a source of 60 electricity.

N is the cathode or negative pole, connected by the conductor n with a source of electricity. This cathode consists of a comparatively large plate of carbon supported upon 65 suitable insulators at the bottom of the cylinder A, below the stand-pipe B.

H is an outlet or overflow pipe for the escape of pulp, &c.

The operation is as follows: The ore reduced to the desired degree of fineness is introduced into the hopper or funnel Q, and a fluid-vehicle used to facilitate its passage to the body of mercury below. Water or even air pressure may be used as such a vehicle. 70 The tank F is supplied with a solution of sodium salt, such as sodium chlorid, (common salt,) which descends through the pipe E to the level of the mercury in the tank A. The electricity being turned on, sodium is formed 75 in the immediate presence of the mercury and is immediately taken up or absorbed thereby. It is obvious that the natural tendency of the pulp, owing to the height of the stand-pipe B, will be to force itself into the body of 80 mercury above the cathode N, after which the greater specific gravity of the mercury will tend to force the pulp-gangue upward into the space above the mercury to escape through the overflow-pipe H. This action is retarded 85 by the plates, which cause the pulp to deviate constantly from a straight line of passage by reason of the fact that the perforations in the adjoining plates do not coincide. This action is further augmented and a thorough 90 admixture of the pulp and mercury assured by the rotation of the plates D with the tube B. By this means it is rendered practically impossible for any of the metal to escape without exposure to and contact with the mercury, 95 and as the latter is kept bright and active by the presence of the newly-formed sodium

the percentage of amalgam attained is largely increased. As the pulp rises above the level  $m m$  of the mercury it is thoroughly stirred and agitated by the rods  $d$  on the disk  $D'$ , thereby disengaging any mercury that may have risen with the pulp and allowing it to fall back into the body of mercury below. The exhausted pulp escapes through the pipe  $H$ . It is well known that mercury will take up or absorb sodium and that water will decompose and separate it from the mercury. Thus the sodium formed on the cathode in the bottom of the cylinder  $A$  will rise with the mercury until decomposed by water, the presence of the sodium keeping the mercury clean and active and in the best condition possible for forming an amalgam of the ore contained in the pulp. The constant formation of fresh sodium at the cathode and its continuous decomposition by the water present is the important practical advantage attained, since if the sodium remained in the mercury it would cause the mercury to grow hard and crusty, and thereby destroy its receptiveness for the metal. Thus it will be seen that it is the actual generation or formation of the sodium directly within the mercury that is the important and distinguishing feature of my invention, the sodium in its nascent state being much more active and effective in preventing the "fouling" or "flowering" of the mercury than when introduced in any other manner. The constant removal of the sodium by decomposition before it deteriorates in efficiency and the continuous formation of fresh active sodium at the cathode keep the mercury-bath constant and uniform in character and effectiveness. This, together with the enforced and positive admixture of the pulp with the mercury, insures the elimination from the pulp and the combination with the mercury of practically all the metal in the pulp if the latter has been reduced to a sufficient degree of fineness. This result is

largely contributed to by the perforated disks  $D$ , which thoroughly break up the mass of ore in the pulp by causing it to pass through the numerous holes in the plates, deviating in its course in doing so. The motion of the plates also retards the upward flow of the pulp and has a scouring effect on the ore therein, making it more receptive to the mercury.

It is to be understood that while I have herein described the use of anodes and cathodes of carbon other suitable substances may be used for the electric terminals.

What I claim as my invention, and desire to secure by Letters Patent, is—

In an amalgamating apparatus for continuously producing sodium amalgam and amalgamating ores under hydrostatic pressure, the combination of a stationary amalgamating-tank  $A$ , adapted to contain mercury, the rotatable stand-pipe  $B$ , provided with perforated disks  $D$ ,  $D$ ,  $D'$ , the cathode  $N$ , situated below the end of said supply-pipe  $B$ , the pipe  $E$ , opening into the amalgamating-tank  $A$ , in proximity to the cathode  $N$ , and considerably below the mercury-level, whereby the ore introduced into the mercury through the pipe  $B$ , is subjected to hydrostatic pressure, the vessel  $F$ , connected with the pipe  $E$ , above the level of the mercury in the amalgamating-tank  $A$ , and the anode  $P$ , situated in said vessel  $F$ , whereby a continuous supply of sodium amalgam is formed at the surface of the mercury in the pipe  $E$ , and diffused through the mercury in the tank  $A$ , by hydrostatic pressure and the agitation thereof caused by the submerging feed,  $B$ , and the rotation of the disks  $D$ ,  $D$ ,  $D'$ , substantially as herein shown and described.

CALEB G. COLLINS.

Witnesses:

D. W. GARDNER,  
GEO. WM. MIATT.